

## UNITED STATES PATENT OFFICE

2,097,239

## ABATING FOAMINESS IN GLUES

Lawrence Bradshaw, Bainbridge, N. Y.

No Drawing. Application April 23, 1935,  
Serial No. 17,853

11 Claims. (Cl. 134—23.8)

This process has for its object the abatement or prevention of foam in glues prepared from proteinous substances such as vegetable seed meals, with or without milk casein, blood albumen and the like.

It is known that glues made, for example, from vegetable seed meals such as peanut meal, with or without the admixture of casein and/or blood albumen, together with lime and alkalies or salts which in the presence of water, can produce free alkalies, frequently have an undesirable tendency to foam upon being mixed with water, especially when the dry ingredients have been mixed together and kept in storage for a considerable time or exposed to unfavorable conditions of temperature and humidity. Foamy glues, from whatever source, are usually deficient in mobility and cohesiveness, do not spread readily and evenly, and when applied to wood veneers and the like give inferior joints.

The present invention relates to a method of abating or preventing foaming and improving the general character of such foamy glues, and also includes mixtures (glue bases) as hereinafter described. The method consists in adding to the dry glue base certain soluble salts or other substances which I have found to possess marked foam-abating properties. Such substances (one or several) are, in general, preferably incorporated in a dry state in the dry glue base, but may be added to the water in which the glue is to be dissolved, or may be added in the dry form or in an aqueous solution to the glue at any appropriate stage of the process of dissolving the glue. I have found that, of the large number of water-soluble substances commercially available, comparatively few possess the foam-abating property in marked degree, while some are entirely devoid of this property. As examples of the former may be mentioned the acetates and formates of calcium, barium, strontium, copper, and manganese, while examples of salts which appear to have practically no anti-foam value are the nitrates and citrates of sodium and potassium.

One method of determining approximately the relative potency of such salts in abating foam is as follows—a weighed amount of the given glue is added to a suitable known amount of water and stirred for 20 minutes in a glue kettle provided with a stirring device rotating at a fixed slow speed, say 60 revolutions per minute. At the end of this time the weight of a standard volume of the glue (say 100 c. c.) is determined. The glue in the kettle is then subjected to a vigorous beating or whipping by rotating the mixer at

double speed for ten minutes. During this period the volume of the glue may increase considerably, due to foaming. At the end of the beating period a second sample of 100 c. c. of the glue is weighed, and the decrease in weight determined, and calculated as a percentage of the weight of the original glue. The greater the amount of foam, the greater will be the percentage loss of weight of the standard volume of glue. In a second test a mixture of 98 parts of the glue with 2% of the selected substance, e. g. a soluble salt (together making 100 parts) are added to the same amount of water as before, and stirred for 20 minutes (the same procedure and same proportion of glue base to water being used as in the first test) and the weight of the standard volume of glue determined. The glue is then beaten as before and a second sample weighed and the percentage loss of weight determined. The difference between the percentage loss of weight in the two cases is a measure of the foam-abatement produced by the particular salt in the beating process.

In the same way, by using equal weights of several different salts respectively in different lots of the same glue their relative foam-abating power (in that particular glue) can be roughly determined.

As examples of the application of this test the following may be given. It may be noted that where sodium fluoride is mentioned in these examples, a commercial sodium fluoride made slightly alkaline with sodium carbonate was used, which in aqueous solution is feebly alkaline to litmus. The calcium acetate used in these tests was the chemically pure salt which when dissolved in water reacts alkaline to litmus, but a less pure, commercial grade is also effective.

## Example 1

The glue base consists of 47 parts of soymeal, 46 parts cottonseed meal, 5 parts milk casein and 2 parts trisodium phosphate. 100 parts of this base are dissolved in water with the aid of 7 parts of lime and 9 parts of caustic soda, with the subsequent addition of 30 parts of sodium silicate solution. A convenient mixing procedure is as follows: To 300 parts of water at about 70° F. in the glue kettle add 100 parts of the glue powder and stir for two minutes. Add 7 parts of lime suspended in 25 parts of water and stir for ten minutes. Add 9 parts of caustic soda dissolved in 25 parts of water and stir two minutes. Add 30 parts of sodium silicate solution (e. g. "water glass" of 41° Bé. which contains about 36% 55

of silicate and about 64% of water), and stir four minutes. Dilute with 30 parts of water and stir two minutes. The mixing is completed in twenty minutes. Total water (in addition to that present in the water glass, about 19.2 parts) 380 parts. In the above operation the stirrer rotated at 60 R. P. M. A portion (100 c. c.) of the glue thus prepared was weighed.

The glue in the kettle was then subjected to 10 beating (i. e. stirring at 120 R. P. M.) for 10 minutes, after which a second 100 c. c. sample was weighed. The percentage decrease of weight was found to be 20%.

In a second test, two parts of strontium acetate 15 were blended with ninety-eight parts of the aforesaid glue base and the mixture dissolved and beaten as before. The percentage decrease of weight amounted to 5.3%, (as compared with the 20% decrease without the strontium acetate 20 added) showing that the strontium acetate has a strong foam-abating action. The difference between 20% and 5.3% namely 14.7%, indicates the reduction in the amount of foam.

Among other salts which exhibit this property 25 in marked degree as indicated by the above method, when they are used in place of an equal weight (2%) of strontium acetate, may be mentioned copper acetate, which gives a percentage decrease of 3.3%, and calcium formate 6.4%.

30 The foam-abating power of various salts differs very considerably but any salt which when mixed into this glue in the manner described produces a percentage decrease of weight (as determined by the aforesaid method) of less than 20% is considered to be an anti-foaming agent, while salts which give a foam value exceeding 20% obviously possess no foam-abating value in this glue, and may even serve to increase the foaminess. Examples of the latter are sodium sulphite and 40 potassium chromate, the addition of which materials, in the above method, were accompanied by decreases in weight, respectively of 21.0% and 24.3%.

It will be understood that these figures were 45 obtained with the particular glue described, and any change in the composition of the said glue, such as the substitution of peanut meal for soy-meal or cottonseed meal, or the use of a more foamy or less foamy soymeal or peanut meal or 50 the use of a greater or lesser amount of casein, or of blood albumen, or the use of different kinds or amounts of the alkali used in dissolving the glue, may change the figures. By way of illustration other examples of glues may be given.

#### 55 Example 2

Soymeal 45 parts, peanut meal 45 parts, blood albumen 10 parts. This glue base was dissolved using the same chemicals and with the treatment 60 as described under Example 1, as far as the stage of dilution with water, at which stage 50 parts of water were added in place of the 30 parts used in Example 1. Total water 410 parts. (With this particular glue base, this amount of water was 65 needed to give the consistency and flow desired). In the foam test the percentage decrease of weight was found (without a foam abating agent added) to be 27.3%. When 2 parts of calcium acetate was incorporated into the glue base (as 70 foam abating agent) and the glue dissolved and subjected to beating in precisely the same way, the percentage decrease of weight was only 14.6%. The difference between 27.3% and 14.6%, namely 75 12.7%, represents the improvement.

#### Example 3

Soymeal 60 parts, peanut meal 38 parts, trisodium phosphate 2 parts. Proceed as in Example 2, using the same chemicals. Total water 5 410 parts. The value obtained in the foam test was 43.6% which was reduced to 28.2% when 2 parts of calcium acetate were mixed into the dry glue base.

#### Example 4

10 Soymeal 96 parts, lime 4 parts. To 300 parts of water at about 70° F. add 100 parts of glue base. Stir about 8 minutes. Then add 9 parts of caustic soda, in 25 parts water, stir 3 minutes. Add 15 parts sodium silicate solution (of about 15 41° Bé), stir 2 minutes. Add 2½ parts of a mixture of equal volumes of carbon disulphide and carbon tetrachloride, stir 5 minutes. Dilute with 65 parts water, stir 2 minutes. Total water 20 390 parts (in addition to that present in the water glass). In the foam test this glue showed a percentage decrease of weight of 40.4, which was reduced to 23.8 when 2% of calcium acetate was incorporated in the glue base.

#### Example 5

25 Casein 50 parts, peanut meal 20 parts, lime 18 parts, sodium carbonate 10 parts, calcium acetate 2 parts. 100 parts of this glue base were added to 250 parts of water at about 60° F. and 30 stirred for about 5 minutes. The mass was then allowed to rest for about 30 minutes and finally stirred for about 5 minutes. In the foam test this glue gave a value of 19.0%. With the calcium acetate omitted, the value was 23.0%. This 33 example represents a casein-lime glue with only a comparatively small proportion of peanut meal added, i. e. the meal was two-fifths of the casein used.

#### Example 6

40 Peanut meal 68 parts, lime 17 parts, sodium carbonate 7 parts, trisodium phosphate 4 parts, sodium fluoride 4 parts. 100 parts of the glue powder are stirred with 300 parts of water at 45 about 70° F. for twenty minutes. In the foam test the value 37.6% was obtained, which was reduced to 32.6% by the incorporation of 1 part of calcium acetate in the dry mix.

#### Example 7

50 The composition of the glue base and procedure used in dissolving it were the same as in Example 1, except that the sodium silicate was omitted. Total water 380 parts. The value obtained in the foam test was 16.3%. When 2 parts of calcium acetate were blended into the glue base the value obtained was 8.8%.

55 The anti-foam salts are effective not only in glues in which free caustic soda is used as a solvent (as in Examples 1 to 4) but also in glues where (as in Examples 5 to 7) alkaline salts such as sodium carbonate, trisodium phosphate and similar alkalis are employed. The anti-foam compounds named in this specification show the strongest effect in glues of which the proteinous component of the adhesive base consists largely of vegetable seed meals. In glues rich in casein or blood albumen and which contain only minor amounts of the proteinous meal, the abatement 60 of the foam is less pronounced.

65 No claim is made herein to the glues mentioned herein by way of example or to other glues containing vegetable seed meal, milk casein or blood albumen, which do not include the use of foam- 70 75

abating compounds of the groups specified herein.

The invention is not limited to adding the foam-abating salts as such, but includes salts which may be formed within the glue by the interaction of basic and acidic substances capable of reacting to form such salts. Thus, I have found that a part of the free lime used in Example 1, may be neutralized in the glue by the addition of an acid such as acetic acid, forming calcium acetate in situ. Thus in the mixing procedure given above, an appropriate amount of the acid (preferably diluted with water) may be added in the kettle at a suitable stage, for example just after adding the lime. In another modification of the process an excess of lime may be used to provide for the formation of a calcium salt within the glue when the acid is added. Naturally the amount of acid used must not be sufficient to completely neutralize the lime and precipitate the glue. In practice, from 1 to 2% of acid has been found to be sufficient. This method however, is less effective than that in which the foam-abating salt is incorporated into the glue base before this is wetted, or the modifications in which the salt is added to the water before the glue base or shortly after the glue base.

Solid acids, such as benzoic, citric or sulfanilic acids added to the glue, for example after mixing with water (excess lime or other alkali preferably being present) are also to some extent, effective in abating foam.

As an example of my preferred method the following may be given: About 2 parts of the salt selected, say calcium formate or acetate, are thoroughly mixed with about 100 parts of the dry glue base. The base given in Example 1 is suitable. The mixture may then be dissolved as described in Example 1. It will be understood that any suitable method of mixing the glue can be used, depending upon the particular glue base.

This example is given by way of illustration only. It will be understood that the amount of anti-foam salt to be used is not limited but may be greater or less depending upon the foaming properties of the base used and the potency of the salt selected and its general chemical character. If highly hygroscopic salts are used, they are preferably added to the water in which the glue is to be dissolved, either as solids or as solutions.

In practice it is advantageous to make up the glue base in such a way that the dissolving operation will be as simple as possible, whereby liability to error in the glue-mixing operation is reduced. This is an added advantage for incorporating the salts used to abate foam, during the making of the dry glue base.

Without limiting the invention to the compounds herein specified, I give below a list of the more important salts and acids which I have found to possess the property of abating foam in glues of the type above mentioned: The acetates, formates, butyrates, and propionates of Al, (NH<sub>4</sub>), Cd, Ca, Cu, Fe, Pb, Mg, Mn, Ni and Sr; ammonium benzoate; barium acetate, formate and tartrate; and calcium lactate, malate and citrate. Of the salts, those of the metals Ca, Sr and Ba (i. e. the alkaline earth metals) with the acid radicals acetic or formic, are preferred, these being considerably more effective than the others given. Of the solid acids which may be added to the glue base containing lime, benzoic and citric are preferred. The present application has

been restricted to the use of salts of organic acids.

The term "foam-abating salt" as used in this case is intended to embrace the above mentioned salts and also salts produced by the interaction of the above mentioned free acids with lime and/or other alkalies present in the glue base or added thereto during the glue-dissolving operation. The term "an alkaline substance" is intended to embrace one or a plurality of alkaline substances. The term "a salt" likewise is intended to cover one or several of the salts of the types indicated.

I claim:—

1. A process of preparing a liquid glue free from an excessive amount of foam, from a base containing a substantial proportion of a proteinous seed meal, which base if agitated with water in the absence of foam-abating agents, would exhibit a tendency to produce foam, which process includes the herein described step of adding a foam-abating salt selected from the group consisting of the water-soluble organic acid salts of aluminum, ammonium, barium, calcium, copper, iron, lead, manganese, nickel and strontium.

2. A dry glue base comprising a proteinous seed meal constituting at least a substantial proportion of the proteinous component of said base, and which base would, in the absence of foam-abating agents, show a substantial tendency to the formation of foam when being mixed with water, together with a foam-abating salt selected from the organic acid salts of aluminum, ammonium, barium, calcium, copper, iron, lead, manganese, nickel and strontium.

3. A dry glue base as in claim 2, in which the foam-abating salt is substantially white.

4. A dry glue base containing a proteinous seed meal as a large component, together with an organic acid salt of an alkaline earth metal, the glue base being one that, in the absence of said organic acid salt would exhibit a tendency to produce a foamy glue when mixed with water.

5. A liquid glue containing the reaction products of a proteinous seed meal with an alkali, together with a soluble acetate of an alkaline earth metal, the latter acting as a foam abater.

6. A dry glue base containing a proteinous seed meal as a large component, together with an acetate of an alkaline earth metal.

7. A dry glue base containing a proteinous seed meal as a large part at least of its proteinous component, which base if mixed with water without a foam-abating agent, would exhibit a tendency to the formation of foam, said base also containing calcium acetate as a foam-abating agent.

8. A dry glue base containing proteinous seed meal as a substantial component, which also contains lime and a free solid acid capable of reacting with lime when water is added, to form a water-soluble calcium salt.

9. A dry glue base as in claim 2, in which the foam abating salt is a soluble non-hygroscopic calcium salt of an organic acid.

10. A process as in claim 1 in which the foam-abating salt specified therein is a salt of a bivalent metal.

11. A process as in claim 1 in which the foam-abating salt specified therein is a salt of a metal having an atomic weight between about 52 and about 66.

LAWRENCE BRADSHAW.